# EUROPEAN PATENT SPECIFICATION

(11) **EP 0 368 338 B1**
(45) Date of publication and mention of the grant of the patent: **22.02.1995**
(21) Application number: 89120887.8
(22) Date of filing: 10.11.1989
(51) Int. Cl.: D06M 15/277, D06M 13/148

(54) **Water-and oil-repellent composition**
Wasser und Öl abweisende Zusammensetzung
Composition repoussant l'eau et l'huile

(30) Priority: 11.11.1988 JP 286376/88; 16.12.1988 JP 319130/88
(43) Date of publication of application: 16.05.1990
(73) Proprietor: DAIKIN INDUSTRIES, LIMITED, Osaka-shi, Osaka-fu (JP)
(72) Inventor: Amimoto, Yoshio, Takatsuki-shi Osaka-fu (JP); Enomoto, Takashi, Settsu-shi, Osaka-fu (JP); Hayashi, Kazunori, Settsu-shi Osaka-fu (JP)
(74) Representative: Hansen, Bernd, Dr. Dipl.-Chem.

(56) References cited:
- FR-A- 2 256 281
- GB-A- 1 222 614

## Description

The present invention relates to an economical water- and oil-repellent composition having good water- and oil-repellency.

A water- and oil- repellent having a fluoroalkyl group has better properties than other conventional water-and oil-repellent, and is widely used. However, it is relatively expensive. In order to decrease the cost, it is proposed to replace a part of the water- and oil repellent having the fluoroalkyl group with a cheap acrylic acid base polymer or polyhydric alcohol such as sorbitol and lactose while keeping the water- and oil-repellency (cf. Japanese Patent Publication Nos. 22487/1963, 8579/1966 and 4160/1978). Although reduction of the cost is achieved to some extent while keeping the water- and oil- repellency, the above proposal is not satisfactory.

FR-A-22 56 281 discloses an oil and water repellent composition containing a fluoroalkyl polymer and glycerol compounds as surfactants. GB-A-1 222 614 discloses a combination of fluorocarbons with an organic glycol as surfactant.

An object of the present invention is to provide an economical water- and oil-repellent composition having sufficient water- and oil-repellency.

This and other objects of the present invention are achieved by a water- and oil-repellent composition which comprises a water- and oil-repellent composition which comprises a water- and oil-repellent which is a homopolymer of an acrylate or methacrylate having a fluoroalkyl group having 4 to 21 carbon atoms or a copolymer thereof with a monomer having no fluoroalkyl group and a glycerol compound selected from glycerol, an ester derivative of glycerol prepared by esterifying a hydroxyl group at the alpha-position with a monoalkane acid having 1 to 6 carbon atoms, an ether derivative of glycerol prepared by substituting a hydrogen of a hydroxyl group at the alpha-position with an alkyl group having 1 to 6 carbon atoms and polyglycerol, said polyglycerol having a melting point of lower than 70°C.

The ester derivative of glycerol is an ester prepared by esterifying a hydroxyl group at the α-position with a monoalkane acid having 1 to 6 carbon atoms, for example, glycerol α-monoacetate, glycerol α-monoformate and glycerol α-mono-n-hexanoate. The ether derivative of glycerol is an ether prepared by substituting a hydrogen of a hydroxyl group at the α-position with an alkyl group having 1 to 6 carbon atoms, for example, glycerol α-monomethyl ether, glycerol α-monoethyl ether and glycerol α-monoisopropyl ether.

In the composition of the present invention, a ratio of the glycerol compound to the water- and oil-repellent is not critical and varies in a wide range dependent on other conditions such as the kinds of the water- and oil-repellent and the glycerol compound. When the amount of the glycerol compound is too large, the water-and oil-repellent composition has deteriorated properties. When the amount of the glycerol compound is too small, the cost is not reduced and the water- and oil-repellency is not improved. Accordingly, the glycerol compound is usually used in an amount of 0.05 to 7 parts by weight, preferably 0.1 to 4 parts by weight per one part by weight of the water- and oil-repellent.

The amount of the water- and oil-repellent having the fluoroalkyl group is not limited. The water- and oil-repellent having the fluoroalkyl group is usually used in an amount of 0.1 to 1.0 per 100 parts by weight of a medium.

The water- and oil-repellents are a homopolymer of an acrylate or methacrylate having a fluoroalkyl group having 4 to 21 carbon atoms and a copolymer thereof with a monomer having no fluoroalkyl group (cf. for example, Japanese Patent Publication 8068/1985).

Preferable acrylate and methacrylate having the fluoroalkyl group are as follows:
R_{f}(CH₂)ₘOCOCR¹=CH₂ and
R_{f}SO₂NR²(CH₂)ₘOCOR¹=CH₂
wherein R_{f} is a perfluoroalkyl group having 4 to 21 carbon atoms, R¹ is hydrogen or a methyl group, R² is an alkyl group having 1 to 10 carbon atoms, and m is an integer of 1 to 10.

Specific examples of the acrylate and methacrylate having the fluoroalkyl group are as follows:
CF₃(CF₂)₇(CH₂)₁₁OCOCH=CH₂
CF₃(CF₂)₄CH₂OCOC(CH₃)=CH₂
CF₃(CF₂)₆(CH₂)₂OCOC(CH₃)=CH₂
CF(CF₃)₂(CF₂)₆(CH₂)₃OCOCH=CH₂
CF(CF₃)₂(CF₂)₁₀(CH₂)₃OCOCH=CH₂
CF₃(CF₂)₇SO₂N(C₃H₇)(CH₂)₂OCOCH=CH₂
CF₃(CF₂)₇SO₂N(CH₃)(CH₂)₂OCOC(CH₃)=CH₂
CF(CF₃)₂(CF₂)₆CH₂CH(OH)CH₂OCOCH=CH₂
CF(CF₃)₂(CF₂)₆CH₂CH(OCOCH₃)OCOC(CH₃)=CH₂
CClF₂(CF₂)₁₀CH₂OCOC(CH₃)=CH₂
H(CF₂)₁₀CH₂OCOCH=CH₂
In addition to the above, the monomer having the fluoroalkyl group of the formula:

CF(CF₃)(CClF₂)(CF₂)₇CONHCOOCH=CH₂

can be used alone or in addition to the above methacrylate or acrylate.

Specific examples of the monomer having no fluoroalkyl group are ethylene, vinyl acetate, vinyl fluoride, vinyl chloride, vinylidene fluoride, vinylidene chloride, acrylonitrile, styrene, α-methylstyrene, p-methylstyrene, acrylic acid and alkyl esters thereof, methacrylic acid and alkyl esters thereof, acrylamide, diacetone acrylamide, methylol diacetone acrylamide, methylol diacetone methacrylamide, vinyl alkyl ether, vinyl alkyl ketone, butadiene, isoprene, chloroprene, glycidyl acrylate and maleic anhydride. The monomer having no fluoroalkyl group is usually used in an amount of 0 to 75, preferably 20 to 65 parts by weight per 100 parts by weight of the polymer.

The homopolymer and copolymer of the above acrylate and methacrylate nay be prepared by bulk polymerization, solution polymerization or emulsion polymerization. The emulsion polymerization is usually preferable. Accordingly, the medium is usually water. The emulsion polymerization uses no specific procedure. For example, as described in Japanese Patent Publication No. 8068/1985, a mixture of monomers is emulsified in the presence of a surfactant and a polymerization initiator, and then polymerized at 50 to 100°C with stirring. The initiator includes a peroxide, an azo compound and a persulfate. As the surfactant, any of anionic, cationic and nonionic surfactants can be used. A mixture of at least one cationic surfactant and at least one nonionic surfactant is preferable.

The composition of the present invention may include conventionally used additives, for example, a crosslinking agent, an antistatic agent, a dye fixing agent, an anticrease agent, a flame retardant, a mothproofing agent and the like, and it may include general-purpose organic solvents, for example, isopropanol and the like.

The water- and oil-repellent composition of the present invention may be applied on a material to be treated by conventionally known methods such as spraying or dipping.

The materials to be treated include natural and synthetic fibers and textiles. The adsorption amount of the water- and oil-repellent to the material to be treated is preferably 0.01 to 2% by weight based on the material to be treated.

When a polyhydric alcohol, an ester or ether derivative of the polyhydric alcohol, or polyglycerol having the melting point of not lower than 70°C which is not included in the glycerol compound of the present invention is used in the water- and oil-repellent composition, an effect is observed to some extent but various defects arise. For example, the ester or ether derivative of a polyhydric alcohol having more carbon atoms or hydroxyl groups than glycerol remains in a cloth in a large amount after the water- and oil-repellency treatment, and the water- and oil-repellency property decreases due to hydrophilic hydroxyl groups and lipophilic alkyl groups. In addition, the treated cloth has deteriorated feeling. An ester or ether derivative of a polyhydric alcohol or alcohol having fewer carbon atoms or hydroxyl groups than glycerol cannot increase the water- and oil-repellency. The polyglycerol having the melting point of not lower than 70°C has the same defects as above.

The water- and oil-repellent composition according to the present invention is economical since the glycerol compound used as the blending component is more easily available than the conventional blending component which comprises the acrylic resin.

In addition, when the conventional water- and oil-repellent is added in a small amount, the water- and oil-repellency is usually insufficient. But, according to the present invention, the water- and oil-repellency is sufficient because of the use of the glycerol compound even if the water- and oil-repellent adheres to a cloth in a small amount.

The present invention will be illustrated by following Examples. The Examples, of course, do not restrict the present invention.

The water- and oil-repellent composition was evaluated as follows:
The water repellency is expressed by the water repellency No. of Table 1 determined by the spray method according to JIS (Japanese Industrial Standard) L-1092. Oil repellency is expressed by the oil repellency No. of Table 2 determined by dropping several drops (diameter: about 4 mm) of a test solvent on two positions of a surface of a test cloth and observing whether the drops are held on the surface for 30 seconds or not. The superscript "+" to the water repellency No. represents that the result is slightly better than said water repellency No.

Feeling is evaluated by measuring the rigidity and softness of the cloth by the Handle-O-meter method according to JIS L-1096.

Resistance to washing is expressed by the water-and oil-repellency Nos. which are determined after carrying out five cycles each consisting of washing a cloth treated with the water- and oil-repellent composition at 40°C in water containing 0.3 % by weight of detergent (Zabu-koso XK, manufactured by Kao) with a bath ratio of 1:40 (cloth:washing liquid (g:g)) for 5 minutes by using a domestic washing machine followed by rinsing the cloth for 15 minutes, dehydrating it and drying it at room temperature.

Resistance to dry cleaning is expressed by the water- and oil-repellency Nos. which are determined by washing a cloth treated with the water- and oil-repellent composition at 30°C in tetrachloroethylene by using a Launder-O-meter followed by drying at room temperature and then measuring the water- and oil-repellency.

**Table 1**

| Water repellency No. | State |
|---|---|
| 100 | No wet on the surface |
| 90 | Slight wet on the surface |
| 80 | Drop like wet on the surface |
| 70 | Considerable wet on the surface |
| 50 | Wet over the whole surface |
| 0 | Complete wet of the surface and backface |

**Table 2**

| Oil repellency No. | Test solvent | Surface tension (dyne/cm, 25°C) |
|---|---|---|
| 8 | n-Heptane | 20.0 |
| 7 | n-Octane | 21.3 |
| 6 | n-Decane | 23.5 |
| 5 | n-Dodecane | 25.0 |
| 4 | n-Tetradecane | 26.7 |
| 3 | n-Hexadecane | 27.3 |
| 2 | n-Hexadecane/Nujol (35/65 by weight) | 29.6 |
| 1 | Nujol | 31.2 |
| 0 | Nujol penetrated | |

### Examples 1 to 4 and Comparative Examples 1 to 3

A water- and oil-repellent used in the water- and oil-repellent composition of the present invention was prepared as follows:

The compound (60 g) of the formula:

(CF₃)₂CF(CF₂CF₂)ₙCH₂CH₂OOCCH=CH₂

(mixture of n = 3, 4 and 5 in a weight ratio of 5:3:1), C₁₈H₃₇OOCCH=CH₂ (38 g), CH₂=CHCOOCH₂CH(OH)CH₂Cl (2 g), pure water (250 g), acetone (50 g), n-dodecyl mercaptan (0.2 g) dimethylalkylamine acetate salt (3 g) and polyoxyethylenealkylphenol (3 g) were charged in a flask, and stirred at 60°C for one hour under a nitrogen stream. A solution of azobisisobutylamidine hydrochloride (1 g) in water (10 g) was added and the copolymerization was carried out while stirring at 60°C for 5 hours under the nitrogen stream. According to a gas chromatography, a conversion of copolymerization was not lower than 99%. From this conversion, a ratio of the repeating units of the resultant copolymer was found to be substantially almost the same as a ratio of the charged monomers. The resultant emulsion contained the copolymer in the solid content of 25 %.

The emulsion was mixed with the blending components as shown in Table 3 to prepare water- and oil-repellent compositions.

Test cloths were a polyester finished yarn woven fabric (hereinafter referred to as PE) and a nylon taffeta fabric (hereinafter referred to as N), and were dipped in the above composition for one minute and squeezed between two rolls so as to adjust the water content at 90 % and 50 %, respectively. Then, they were dried at 110°C for three minutes, PE was thermally treated at 180°C for 40 seconds and N was thermally treated at 170°C for one minute to impart the water- and oil-repellency. The water- and oil-repellency of the treated cloths were measured. The results are shown in Table 4.

As is clear from Table 4, when the glycerol compound of the present invention is added to the water- and oil-repellent composition, good water- and oil-repellency is achieved.

**Table 3**

| Example No. | Test cloth | Adhesion of repellent to fabric (wt%) | Blending component | Adhesion of blending component to fabric (wt%) |
|---|---|---|---|---|
| 1 | PE | 0.03 | Glycerol | 0.015 |
| | N | 0.10 | | 0.05 |
| 2 | PE | 0.03 | Glycerol α-monomethyl ether | 0.015 |
| | N | 0.10 | | 0.05 |
| 3 | PE | 0.03 | Glycerol α-monoacetate | 0.015 |
| | N | 0.10 | | 0.05 |
| 4 | PE | 0.03 | Polyglycerol (melting point: 30°C) (molecular weight: 170) | 0.015 |
| | N | 0.10 | | 0.05 |
| Comp.1 | PE | 0.03 | - | - |
| | N | 0.10 | | - |
| Comp.2 | PE | 0.03 | Sorbitol | 0.015 |
| | N | 0.10 | | 0.05 |
| Comp.3 | PE | 0.03 | Polyglycerol (melting point: >70°C) (molecular weight: 1000) | 0.015 |
| | N | 0.10 | | 0.05 |

## Claims

1. A water- and oil-repellent composition which comprises a water- and oil-repellent which is a homopolymer of an acrylate or methacrylate having a fluoroalkyl group having 4 to 21 carbon atoms or a copolymer thereof with a monomer having no fluoroalkyl group and a glycerol compound selected from glycerol, an ester derivative of glycerol prepared by esterifying a hydroxyl group at the alpha-position with a monoalkane acid having 1 to 6 carbon atoms, an ether derivative of glycerol prepared by substituting a hydrogen of a hydroxyl group at the alpha-position with an alkyl group having 1 to 6 carbon atoms and polyglycerol, said polyglycerol having a melting point of lower than 70°C.

2. The water- and oil-repellent composition according to claim 1, wherein the composition contains the glycerol compound in an amount of 0.05 to 7 parts by weight per one part by weight of the water- and oil-repellent.

## Patentansprüche

1. Wasser- und Öl-abstoßende Zusammensetzung, umfassend ein Wasser- und Ölabstoßungsmittel, welches ein Homopolymer ist aus einem Acrylat oder Methacrylat mit einer Fluoralkylgruppe mit 4 bis 21 Kohlenstoffatomen oder ein Copolymer davon mit einem Monomer ohne Fluoralkylgruppe, und eine Glyzerinverbindung, ausgewählt aus Glyzerin, einem Esterderivat von Glyzerin, hergestellt duch Verestern einer Hydroxylgruppe an der alpha-Stellung mit einer Monoalkansäure mit 1 bis 6 Kohlenstoffatomen, einem Etherderivat des Glyzerins, hergestellt durch Substituieren eines Wasserstoffs oder einer Hydroxylgruppe an der alpha-Stellung mit einer Alkylgruppe mit 1 bis 6 Kohlenstoffatomen und Polyglyzerin, wobei das Polyglyzerin einen Schmelzpunkt von weniger als 70°C hat.

2. Wasser- und Öl-abstoßende Zusammensetzung gemäß Anspruch 1, bei der die Zusammensetzung die Glyzerinverbindung in einer Menge von 0,05 bis 7 Gew.-Teilen pro einem Gewichtsteil des Wasser- und Ölabstoßungsmittels enthält.

## Revendications

1. Composition repoussant l'eau et l'huile qui comprend un répulsif vis-à-vis de l'eau et de l'huile qui est un homopolymère d'un acrylate ou d'un méthacrylate possédant un groupement fluoroalkyle en C₄-C₂₀ ou un copolymère de celui-ci avec un monomère ne contenant pas de groupement fluoroalkyle et d'un composé du glycérol choisi parmi le glycérol, un dérivé ester de glycérol préparé par estérification d'un groupement hydroxyle en position α à l'aide d'un acide monoalcanoïque en C₁-C₆, un dérivé éther du glycérol préparé par substitution d'un atome d'hydrogène du groupement hydroxyle en position α par un groupement alkyle en C₁-C₆ et un polyglycérol, ledit polyglycérol ayant un point de fusion inférieur à 70°C.

2. Composition repoussant l'eau et l'huile selon la revendication 1, dans laquelle la composition contient le composé du glycérol à raison de 0,05 à 7 parties en masse par partie en masse du répulsif vis-à-vis de l'eau et de l'huile.
